

W. McA. JOHNSON.

## METHOD OF ELECTRICALLY SMELTING VOLATILE METALS.

APPLICATION FILED JAN. 17, 1911.

1,080,912.

Patented Dec. 9, 1913.

3 SHEETS—SHEET 1.



Witnesses:

Henry Ryan

Montgomery

Woolsey McJohnson Inventor  
By his Attorney  
Dens. Warfield & Dens.

W. McA. JOHNSON.

METHOD OF ELECTRICALLY SMELTING VOLATILE METALS.

APPLICATION FILED JAN. 17, 1911.

1,080,912.

Patented Dec. 9, 1913.

3 SHEETS—SHEET 2.



WITNESSES

Henry Ryan  
Henry Ryan

INVENTOR

W. McA. Johnson  
BY  
Dens, Wadfield & Dens  
ATTORNEY

W. McA. JOHNSON.  
METHOD OF ELECTRICALLY SMELTING VOLATILE METALS.  
APPLICATION FILED JAN. 17, 1911.

1,080,912.

Patented Dec. 9, 1913.

3 SHEETS—SHEET 3.



Witnesses:  
Henry Ryan  
John W. Berry

# UNITED STATES PATENT OFFICE.

WOOLSEY M.C.A. JOHNSON, OF HARTFORD, CONNECTICUT.

## METHOD OF ELECTRICALLY SMELTING VOLATILE METALS.

1,080,912.

Specification of Letters Patent.

Patented Dec. 9, 1913.

Application filed January 17, 1911. Serial No. 603.

To all whom it may concern:

Be it known that I, WOOLSEY M.C.A. JOHNSON, a citizen of the United States, residing at Hartford, in the county of Hartford and 5 State of Connecticut, have invented certain new and useful Improvements in Methods of Electrically Smelting Volatile Metals, of which the following is a full, clear, and exact description, such as will enable others 10 skilled in the art to which it appertains to make and use the same.

This invention deals with certain improvements in the art of obtaining from their ores or compounds, metals volatilizing at 15 their smelting temperatures, but inasmuch as certain noteworthy characteristics of the invention prominently appear in its more intense aspect as a method of reducing and separating zinc by a volatilizing process in 20 which, through the instrumentality of an electric furnace, the vapors of zinc, together with portions of the charge, are advantageously utilized as conductors of an electric current; it will be conducive to clearness to 25 specifically disclose this invention by way of such embodiment thereof.

Now this invention has in contemplation the formulation of an essentially commercial method of deriving metallic zinc from its 30 ores or compounds through the instrumentality of an electric furnace, and it seeks so to devise and coördinate the several steps of this process that each step will not only be effective in its specific purpose, but also 35 will harmonize and coöperate with the other steps in enhancing the general efficiency of the complete method.

Another and further object is to render 40 commercially available a complete zinc-smelting process capable of a continuous operation in the treatment of large quantities of varied classes of zinc ores with a small labor charge, at a high thermal efficiency, with a low cost of repairs and requiring 45 the investment of only a moderate amount of capital, and which will be capable of yielding directly merchantable products and by-products such as pure spelter, lead-copper matte, base lead bullion, and 50 sulfur-bearing gases available for the production of sulfuric acid, if desired.

To promote a full understanding as to 55 the manner in which this process may be commercially applied and best adapted for the specific treatment of zinc-bearing ores, drawings exemplifying a preferred embodiment

of a preferred means instrumental in carrying out certain steps of this process have been appended as a part of this disclosure, and in such drawings like characters of reference denote corresponding parts 60 throughout the several views, of which,

Figure 1 is a top plan view of an electric furnace such as I contemplate using, preferably in connection with sulfur-bearing 65 ores of zinc which have first been treated as outlined in my United States Patent No. 868,345; Fig. 2 is a longitudinal vertical section taken through said furnace showing the hoppers in section and omitting certain 70 parts for clearness; and Fig. 3 is a vertical transverse section taken along line 3—3 of Fig. 1 looking toward the left hand side thereof.

Continuing now by way of a detailed description of the method proposed in accordance with my invention, it will be convenient to describe the structural details of this apparatus while tracing the successive steps pursued in carrying out my method especially as applied to the treatment of zinc 75 ores relatively rich in iron and sulfur.

Turning now to the drawings, A indicates a furnace body which conveniently may be rectangular in contour and be formed of 80 refractory material, such as fire brick, built to form a base portion or bottom 1, a front wall 2, a rear wall 3, two end walls 4 and the top 5. Preferably, the latter will also be made up of fire bricks 6 placed together 85 in the form of an arch to form a strongly constructed roof for the furnace. In order to further enhance the strength of the furnace body, an outer layer 7 of concrete surrounding the uprising walls may be used, 90 and furthermore suitable stays, heavy angle irons, tie rods and the like, may also be employed to strongly bind the whole into a self-contained and mechanically strong structure.

The construction above described provides 95 an inclosed substantially air-tight chamber which may vary in dimensions but which, for example, may be 30" by 60" and high enough to enable it to contain a charge, column about 40" high, in which the charge is 100 to be electrically heated out of contact with the air, and the instrumentality for so heating consists of suitably arranged electrodes one or more of which are depending and another of which may be arranged to lead in, 105 at or near the bottom of the furnace chamber. Thus, an electrode 8 which, for in-

stance, may be made of two copper bars  $\frac{1}{2}$ " by 4", or may be constructed of other suitable material, such as graphite, carbon, or iron, leads through the walls of the furnace and extends toward or near the bottom surface thereof so as to expose a sufficient surface to afford an opportunity for the easy passage of the electric current. Inasmuch as during the normal operation of the furnace, 5 a layer of molten material of extremely high electrical conductivity, such as lead, iron or fusible sulfid, accumulates in the hearth of the furnace, such electrode tends to heat considerably and by reason of the resultant 10 expansion, tends to loosen the joint between such electrode and the material of the furnace body and thus possibly enable this molten material to run out and escape from the furnace. To obviate this, I propose to 15 surround or arrange adjacent portions of the electrode, a cooling means such as the coiled pipe 9, through which water may be circulated to absorb all excessive heat and thus maintain a tight joint in the parts.

20 25 In the drawings, I have also shown a pair of depending carbon or graphite electrodes 10 and 11, but it is to be noted that this invention in this respect is subject to some modification. These electrodes are 30 preferably constructed of some enduring material, such as graphite, capable of conveying large currents. For example, the two upper electrodes can be made 6" square, and so mounted as to permit of being adjusted in 35 position up and down. To this end, I recommend that the upper ends of said graphite electrodes be placed within a contact block 12 which is suspended by means of the chain 13 of the block and falls. Owing to 40 the fact that these electrodes are excellent conductors of heat and thus tend to become highly heated at their upper ends, and in turn overheat the metallic connections, I provide the blocks 12 with one or more interior channels 14 through which cooling 45 water is circulated by means of suitable flexible connections as with rubber hose, as indicated. This simple construction suitably carries the weight of the electrodes and at 50 the same time enables the operator to very easily and rapidly adjust the relation between these electrodes and the bath of slag. The arch of the electric furnace is preferably provided with an aperture for each electrode, 55 preferably having downwardly converging sides, shown by 15. A packing of asbestos 60 forms a simple yet effective gas-tight joint and at the same time does not interfere with the adjustment of such electrodes.

60 65 The electrodes may be connected in various ways, depending upon the character of the ore and reducing agent, and on the voltage that the power plant can most conveniently deliver. Thus, they may be connected in series so that the molten electrode

on the hearth of the furnace will act as an intermediate electrode for receiving the current passing downwardly from one of the upper electrodes and for delivering such current upwardly to the companion electrode. Or the upper electrodes may be placed so as to form an equilateral triangle connecting with a three-phase current, in which case the molten electrode will serve as the neutral conductor. But the improved 70 form of connection, and the one which possesses special advantages and is most preferred for practical purposes, is that shown by the drawings, in which all of the upper uprising electrodes are connected only to 75 one bus-bar of the generator or transformer and the lower electrode is connected to the other bus-bar. The furnace is most advantageously operated by an electrical apparatus capable of furnishing power at a constant amperage, and thus either direct, single phase or polyphase current can be employed. The voltage suitable for my process can 80 conveniently be 110 and the amperage 4500, and a good practical rule is to employ about 600 amperes per square foot of smelting zone to 85 absorb 80 per cent. of the net electric energy directly in the smelting zone, about 18 per cent. in the slag bath, and about 2 per cent. in the carbonaceous filter, which will be 90 shortly described.

95 The crucible of the furnace is first charged with pig lead in such quantity to form, when melted, the lead pool. Then the furnace may be started in various ways within the ordinary skill of the art, as, for example, by preliminarily pouring hot metal or hot slag into the same, or by simply striking an arc by contacting the electrodes with a coke covering carried by the lower electrode and 100 gradually raising it as the slag melts, or a certain amount of slag may be placed in the furnace and the latter then heated by building a wood or coke fire in the same and by 105 utilizing the electric current, as may be desired.

110 Before commencing the regular charging for the continuous smelting operation, I propose that the furnace and its contents be thoroughly heated up to avoid untoward 115 condensations of the metal. In this preliminary heating run, the furnace is charged at intervals with old slag or with a slag-making charge. It is advisable that this slag shall contain no zinc or other volatile element of 120 a nature capable of subsequently condensing to clog up the outlet pipes of the furnace or to accumulate in the condenser. After eight to ten hours of prolonged heating, using something like an average of 200 k. w. on a 125 furnace of 500 k. w. rating, the slag will be heated to 1300 to 1350 degrees C., and the eductor will be heated somewhat above 862 degrees C. by the flow of gas from the slag and by the heat deducted and radiated from 130

the furnace chamber. When these conditions have been attained, the charging pipes are opened and a charge of zinc ore mixed with fine coke or coal and heated to a temperature somewhat above the melting point of zinc, *i. e.*, above 415° C. This charging may take place through one or more charging funnels 17, which may be constructed of fire clay and luted through the arched roof 10 so as to terminate within the same a short distance below said roof. These funnels may be arranged in different locations in the roof, but preferably they are disposed adjacent to the forward wall of the same as a matter of 15 convenience in adding charge thereto. In the construction shown, the funnels 17 are maintained in a heated condition by the hot vapors in the upper part of the furnace, and they may be jacketed above their entrance 20 into the furnace by a preheating device.

It is important, either by introducing the charge in a sufficiently heated state, or by heating the funnels, that the column in such funnels be kept hot enough to enable it to 25 feed properly. In initial runs, when the operators are unused to the operation, it is well to measure the temperature of the first charges by one or more pyrometers 27 disposed somewhat as shown in the drawings, 30 for if the charge be cold and the reduction of ZnO and the evolution of zinc vapor and carbon monoxide be rapid, the charge in the smelting chamber and in the charging pipes will condense zinc in their upper portions 35 so as to disseminate through the charge the zinc as a solid metal in the form of frozen drops. This action will cause a scaffold to form which will later be melted out by the heat from the slag bath which will suddenly 40 drop the cold charge on the heated slag and possibly cause an explosion, depending on the severity of such untoward conditions.

Under normal working conditions I propose that the distance between the slag and the bottom of the overlying electrodes shall be about 8 to 10 inches and thereby put into 45 practical effect my discovery that this is not only metallurgically advantageous, but also commercially feasible by reason of the conductivity of the disseminated iron and the zinc vapor present in the smelting zone, the conductivity of which is marked and appreciable at the temperature existing in the smelting zone, *i. e.*, some degrees above 50 1033° C.

In the case of one specific type of ore which my process is adapted to handle with peculiar advantage, sulfids of zinc, lead and iron are concomitantly present in material 55 quantities. In such case, this invention proposes as a preliminary step in the process the external preparation of such ore in accordance with the plan outlined in my United States Patent No. 868,345, granted 60 October 15, 1907, in accordance with which

such oxides or compounds as PbO, Fe<sub>2</sub>O<sub>3</sub> and FeO · (SiO<sub>2</sub>)<sub>x</sub>, etc., are formed from the sulfids by an outside carefully conducted roasting operation, and said compounds reduced by carbonaceous material in an exterior furnace, so that the prepared and pre-heated charge will contain from 15 to 25 per cent. of sponge iron. The purpose of this step is to obtain a starting material in which further reactions and reductions can take place in a continuous way in the electric furnace. In any event, the charge is continuously introduced into the electric furnace as rapidly as smelted. 70 75

Assuming that the furnace has been brought into a condition of normal operation, its contents will ordinarily be as represented by the drawings, in which 18 indicates a bath or lowermost layer of lead in a molten condition, 19 indicates an overlying layer of matte, and 20 represents a considerable body of fluid slag. Ordinarily the lead pool will be about 2" to 3" deep and preferably a lead well shewn by 23 is luted through the furnace wall, which is provided with a recess 24 underlying the lead well to heat or cool the latter. A tap 26 enables the slag to be run out, and an underlying tap 25 enables a proper amount of matte to be maintained, say from 4" to 8" deep. These taps may be water-cooled and disposed according to circumstances and may serve to drain the furnace whenever this is desirable. The mass of slag is of considerable advantage, inasmuch as it serves in the capacity of a thermal balance wheel, so to speak, and furthermore, may be utilized for the generation of additional heat in the electric furnace by reason of its resistance to the passage of the electric current. The slag bath acts also as an emergency rheostat and gives a definite fixed minimum internal resistance to the furnace that prevents short-circuiting by exaggerated arcing through the zinc vapor. While in normal operation it works as a thermal balance wheel, in periods of need it acts as an electrical balance wheel. The charge 21 will occupy a large portion of the furnace chamber, as shown by the drawings, and between it and the upper surface of the bath of slag a layer, rich in carbon, such as coke 22, may be formed. 90 95 100 105 110 115

When the electric current is passed through the electrodes, its electrical energy will be partly absorbed by the bath of slag 20 and partly in the smelting zone. In said smelting zone the current is conducted partly through some solid contacting portions of the charge, and partly also through the zinc vapor which is present and which is utilized in part as a carrier for the current. 120 125

As the slag bath plays a peculiar part in my process, it is perhaps advisable to am- 130

plify its purpose and its characteristic relation to other parts of the process, to accentuate to those skilled in the art the interdependence of the various steps of my process and the manner in which they promote a smooth and controllable smelting by mutually acting in an automatic compensating capacity. This slag bath operates as a means instrumental in carrying out that part of my process whereby about 18 to 20 per cent. of the total amount of electrical energy is directly and specifically absorbed and transformed by resistance into heat so that as its temperature increases by any means, the heat thrown upward also increases, and as the heat internally gained by the slag bath decreases, its resistance decreases. Thus, as the furnace is operated on constant amperage the voltage of the furnace decreases and a smaller proportion of the total energy is absorbed by the slag bath, and accordingly a nearly constant flow of heat keeps the smelting zone at the proper temperature for the smelting. The heat of any intense and momentary local heating of the smelting zone is absorbed by slag bath. Its great latent heat combined with the cooling effect of the descending charge which has great heat requirements keeps heat supplied to the smelting zone in such degree as to keep the smelting zone at  $+1033^{\circ}$  C., should the temperature there fall below this smelting temperature, and thus the smelting conditions are kept uniform.

The slag is most advantageously made of a lime iron-oxid sesquisilicate with not over 12 per cent.  $Al_2O_3$ , and to increase fluidity I may incorporate in the charge from 5 to 10 per cent. of fluor-spar. This, however, is not essential. I advise the operation of the furnace be such that the slag is kept about 100 degrees C. above its running temperature. This is easily effected by the per cent control over temperature that my electro-thermic smelting process allows. The slag bath continually absorbs the mineral components of the charge in a manner exactly similar the role of slag in a lead or iron blast-furnace.

The foregoing general and detailed description of the functions of the slag bath always must be kept in mind in connection with the following description of the actual smelting operation in the shaft of the furnace. In the smelting zone, as indicated by the lines of force 28 in Fig. 3 of the drawing, the zinc oxid is reduced at  $+1033^{\circ}$  C. and the slag and matte and lead formed and melted. These pass progressively downward and separate according to their specific gravities in the usual manner. The heat for these operations is furnished by the electrothermic effect of the electric current.

The gases of reduction, viz., Zn and CO,

at  $+1033^{\circ}$  C. arising from the smelting zone, percolate upward through the descending charge, thereby heating it, and are at the same time themselves cooled to a few degrees above  $862^{\circ}$  C. (Richards' *Metallurgical Calculations*, Part III, page 622, shows this to be minimum temperature at which equal volumes of Zn and CO can coexist in gaseous state under 760 min. pressure), and pass from the top of the charge column, through the eductor to the condenser. The charge settles downward regularly, being replenished by the fall of fresh charge from the feed pipes to the furnace chamber.

Such is the general smelting operation. To enable one skilled in the art to gain a more practical knowledge of the electro-chemical details of the smelting zone, let us consider the course of a small cube of charge leaving the feed pipe at a temperature of  $+415^{\circ}$  C. As such an element descends, it comes continuously in contact with the gases of reduction ever growing hotter as the element progresses toward the smelting zone and its temperature is raised to the temperature at which the charge is conductive. This critical smelting temperature is about  $950^{\circ}$  C. As soon as the element attains this critical smelting temperature, it has reached, of necessity, the smelting zone. Here the current density of the element increases from zero to an appreciable figure and the electrothermic result is that the element rapidly assumes the reduction temperature for zinc oxid, i. e.,  $+1033^{\circ}$  C. Immediately thereafter the current density through the element of charge again increases for the zinc vapor autogenously generated acts as gaseous conductor. The temperature would rise very quickly much above  $1033^{\circ}$  C. were it not for the great heat-absorbing capacity of the charge, for the reaction  $ZnO + C = Zn + CO$  is strongly endothermic and in the case of pure hot materials with hot products it absorbs per kg. of zinc contents approximately 1500 cal. (See Richards *Met. Calculations*, Part I, page 50).

As a natural result, the reduction proceeds actively and its rate is proportional to the rate at which electrical energy is given to the element of charge, for the reaction velocity of the reduction of the zinc oxid by carbon is a geometrical function of the temperature of the reacting bodies less  $1033^{\circ}$  C. Mathematically expressed, we have  $^vZnO + C = F$  ( $^vZnO + C - 1033^{\circ}$  C.)

Theoretically, with ample electrical energy at hand, immense amounts of  $ZnO + C$  could be reduced in a very short space of time, but, from a practical standpoint, the rate of reduction is limited by the necessity for a progressive and regular descending of the charge, by the maximum allowable con-

80

85

90

95

100

105

110

115

120

125

130

ductance of the electrodes and by the ability to evolve the gases upward through the charge and not downward into the slag.

By effecting the reduction of zinc oxide in a fusion electrothermic zinc process the reacting bodies are in a state of hot solution, and therefore the reduction proceeds from 20 to 100 times as fast as in the zinc retort and the smelting proceeds 2 to 10 times as fast as in a copper-matting furnace.

The above shows the electrochemistry of the smelting zone. The purely electrical action of the smelting operation is partly arcing through the zinc vapor and partly conductance through the solid and liquid particles of the charge. In the smelting zone, the furnace does not operate on the resistance principle of electric smelting or on the arc principle, but on a combination 20 of the two classes of electric smelting operations.

At its surface the slag has a temperature of +1250° C. Which is sufficient for the reactions,  $ZnS + Fe = FeS + Zn$ ,  $ZnO + Fe = FeO + Zn$  to proceed quietly and smoothly. These reactions are not so strongly endothermic as the reduction of zinc oxide by carbon. They absorb both electrical heat and heat radiated and conducted upward from the slag bath.

The proper adjustments in the relative positions of the upper electrodes to the bath of slag can be made in several ways: (1) Electrodes can be raised as slag level raises 35 by any well known mechanical means, such as a differential block. In this case the slag is removed by tapping intermittently. (2) The slag can be tapped continuously and the level of slag bath held constant.

40 The proper relative position and dimensions of electrodes, slag bath and charge to make the smelting most efficient, depend on cost of power, on cost of ore, price of products, character of ore and reducing agent, and on voltage at which power can best be furnished.

In order to carry out my process successfully, the electrometallurgist should pay attention to the subordinate function of the 45 charge. Besides furnishing the material to be smelted and acting with its products as the main resistor, it has three specific sub-functions. (a) It filters out any lead fume and condenses any lead vapor (thereby making a 99.80 per cent. pure spelter) and filters out any of the fumes of silicon, aluminum, and any dust. (b) It fixes any tarry vapor and lessens the clogging up of the condenser by tar. (c) It cools the gases to the 50 temperature best suited for condensation. Thereby the condenser is relieved of work and its capacity accordingly is increased. The transfer of heat units to the descending charge by the upward percolating gases lessens the heat requirements of the smelting

operation. In this way a double advantage is gained, for the amount of electrical energy needed for smelting a charge of given composition is lessened and the capacity of the condenser is enhanced.

In the normal operation of the process, a top layer 30 of carbonaceous material preferably will be used. This may advantageously be introduced through the pipes 31 which pass through the furnace roof adjacent the regular charging funnels 17 and which preferably are arranged so that the carbonaceous material will gravitate around the discharge ends of the funnels and around the depending electrodes. In this way, all vapors must first pass through this reducing medium before leaving the furnace. By using this material in this manner, it is maintained at an effective temperature without employing any heating means other than the furnace, with a resultant economical operation.

The charging of the furnace with the "mix" and also with the charcoal or equivalent material for "super-reducing" can be done either intermittently by directly opening the charge holes of by some apparatus as a double bell and hopper. In the latter case, a plus pressure of some reducing or indifferent gas as hydrogen, carbon monoxide, 90 nitrogen or a mixture of the three as a high grade producer as had best be applied to the charging mechanism in order to prevent the ingress of air to the furnace during the charging operation. But the best and 100 simplest way is to feed the furnace continuously and directly through fire clay or cast iron pipes extending to level of the charge column. To prevent the clogging of these by the condensation of zinc in them 105 to solid form, it is only necessary to insure that the charge in the feed pipes be kept slightly above the melting point of zinc 415° C. according to one of the three following ways: (1) Charging the "mix" hot, above 110 415° C. and below a temperature at which any amount of zinc can coexist with carbon monoxide in the gaseous state, say 500° C. (2) By designing the feed pipe so that the internal heat of the furnace keeps the 115 charge above 415° C. and below 500° C. (3) By jacketing the pipe and surrounding it with an atmosphere of gases above 415° C. and below 500° C. In any event, the frictional resistance to flow of gas of the "mix" 120 in "feed pipes" must be so great that the zinc vapor has the chance to condense on the descending "mix" in the feed pipes, as it is well to make the furnace always strongly exhalant. Any carbon monoxide 125 escaping at the feed pipes can be burnt or it can be collected and used as a gaseous fuel. This facilitates the condensation by enriching the gas, for the liquid zinc is re-volatilized when the charge descends into 130

the smelting zone and finally passes out as zinc vapor through the eductor into the condensing apparatus.

After the mix is charged, a layer of char-  
5 coal is introduced through the appropriate  
charging apertures. This serves several  
purposes. A part of the electrical energy,  
2 per cent., passes through it and present  
local points of arcing, giving rise to carbon  
10 vapor. Thus the reduction of any weak  
oxidizers, such as  $\text{SO}_2$ ,  $\text{CO}_2$  or  $\text{H}_2\text{O}$ , takes  
place. This prevents the oxidization by  
these oxidizers of the zinc vapors in the con-  
15 denser and reduces to a minimum the for-  
mation of blue powder. It also "fixes"  
any heavy tars into lighter hydrocarbon  
that will not, as the heavy tars will, clog  
up the condenser. The reduced vapors  
20 leave the furnace through the eductor  
which is preferably inclined into the fur-  
nace chamber at a relatively steep gradient,  
say 1-3 or 1-4, so that while it may act  
as a collection chamber, it will also allow  
25 such products as may condense therein to  
gravitate back into the furnace and there  
be volatilized. This eductor is so made  
and connected with the condenser, that the  
operator may insert a rabble through the  
30 condenser and push the dust back into the  
smelting chamber. This eductor is heavily  
insulated with mineral wool or asbestos  
incased in sheet iron, so that but little molten  
35 zinc will be condensed therein.

From the foregoing disclosure it will be  
35 perceived that I have succeeded in devising  
an electric zinc smelting method in which  
the various commercial requirements are  
adequately fulfilled and that, while said  
method is essentially simple in character, it  
40 nevertheless is capable of yielding metallic  
zinc of a very high grade and free from the  
impurities which are ordinarily found in  
zinc bullion commercially produced from  
ordinary ores.

45 Without further elaboration, and in the  
light of current knowledge, the foregoing  
disclosure will sufficiently suggest and  
otherwise enable those skilled in this art to  
readily utilize various interchangeably  
50 available and mechanically equivalent steps  
and treatments which, although perhaps cal-  
culated to appear widely different under a  
superficial inspection, and follow in a varied  
sequence, would nevertheless embody cer-  
55 tain, if not all of the herein-described fea-  
tures which, from the aspect of the prior  
art, constitute essential and advantageous  
characteristics of this invention, and there-  
fore such processes should and accordingly  
60 be intended to be comprehended in the  
wording and scope of the following claims.

Having described my invention, what I  
claim as new and desire to secure by Let-  
ters Patent is:

65 1. The method of smelting ores yielding

a volatile metal, which consists in elec-  
trically heating a charge proportioned to  
yield a fusible slag, conducting the volatile  
reaction products into contact with carbon  
heated to its temperature of maximum re-  
70 ductivity, continuously replacing the car-  
bon and condensing the metal, substantially  
as described.

2. A continuous smelting process of the  
nature disclosed, which consists in super-  
posing a heat reducible charge containing  
a volatile metal upon a molten electrode,  
and causing an electric current to pass  
75 through the charge and through the evolved  
metallic vapors, and also through the elec-  
trode.

3. The method of smelting ores yielding  
a volatile metal which consists in progres-  
sively heating, in the absence of extraneous  
air, a charge proportioned to yield a fusi-  
80 ble slag, conducting the volatile reaction  
products through the charge, thereby pro-  
gressively cooling the same, and condensing  
the metal apart from the charge.

4. The method of smelting ores yielding  
a volatile metal which consists in heating,  
in the absence of extraneous air, a charge  
comprising a reducing agent and propor-  
tioned to yield a fusible slag, preventing the  
escape from the charge with the volatilized  
90 metal of an agent capable of combining with  
the volatilized metal, and condensing the  
volatilized metal apart from the charge.

5. The method of smelting ores yielding  
a volatile metal which consists in heating, 100  
in the absence of extraneous air, a charge  
comprising a reducing agent and propor-  
tioned to yield a fusible slag, preventing the  
escape from the charge with the volatilized  
metal of a gaseous agent capable of 105  
combining with the volatilized metal, and  
condensing the volatilized metal apart from  
the charge.

6. The method of smelting ores yielding  
a volatile metal which consists in heating, 110  
in the absence of extraneous air, a charge  
comprising a reducing agent and propor-  
tioned to yield a fusible slag, preventing the  
escape from the charge with the volatilized  
metal of a gaseous agent capable of 115  
oxidizing the volatilized metal, and condens-  
ing the volatilized metal apart from the  
charge.

7. The method of smelting zinc-ores  
which consists in heating, in the absence of 120  
extraneous air, a charge of ore and agents  
having a greater affinity for other elements  
of the volatilized products than for zinc-  
vapor, the charge being proportioned to  
yield a fusible slag, preventing the escape  
125 from the charge with the zinc-vapor of a  
gaseous agent capable of combining with  
the zinc-vapor, and condensing the zinc-  
vapor apart from the charge.

8. The method of smelting zinc-ores

which consists in progressively heating, in the absence of extraneous air, a charge consisting of ore and agents having a greater affinity for other elements of the volatile products than for zinc, the charge being proportioned to yield a fusible slag, conducting the volatile reaction products through the charge, thereby progressively cooling the same, and maintaining the temperature of the charge such as to prevent the escape from the charge of a gaseous agent capable of oxidizing the zinc-vapor, and condensing the zinc apart from the charge.

15 9. The method of smelting ores yielding a volatile metal which consists in heating a charge of ore, carbon, and agents having a greater affinity for other elements of the volatilized products than for zinc-vapor, the charge being proportioned to yield a fusible slag, conducting the volatilized zinc through the charge, preventing the escape from the charge with the zinc-vapor of a gaseous agent capable of combining with the zinc-vapor, condensing the zinc-vapor apart from the charge, and separately collecting such of the products as would combine with the zinc-vapor.

10 10. The method of smelting ores yielding a volatile metal which consists in progressively heating, in the absence of extraneous air, a charge comprising a reducing agent and proportioned to yield a fusible slag, conducting the volatile reaction products through the charge, thereby progressively cooling the same, preventing the escape from the charge of an agent capable of combining with the volatilized metal, and condensing the metal apart from the charge.

15 11. The method of smelting zinc-ores which consists in progressively heating a charge of ore and agents having a greater affinity for other elements of the volatilized products than for zinc-vapor, the charge being proportioned to yield a fusible slag, conducting the volatile reaction products through the charge, thereby progressively cooling the same, preventing the escape from the charge with the zinc-vapor of a gaseous agent capable of oxidizing the zinc-vapor, and condensing the zinc-vapor apart from the charge.

12. The method of smelting ores yielding a volatile metal which consists in progressively heating a charge of ore, carbon, and agents having a greater affinity for other elements of the volatilized products than for zinc-vapor, the charge being proportioned to yield a fusible slag, conducting the volatilized zinc through the charge, thereby progressively cooling the same, preventing the escape from the charge with the zinc-vapor of a gaseous agent capable of

of combining with the zinc-vapor, condensing the zinc-vapor apart from the charge, and separately collecting such of the products as would combine with the zinc-vapor.

13. The method of smelting ores yielding a volatile metal which consists in progressively heating a charge comprising carbon, and proportioned to yield a fusible slag, conducting the volatile reaction products through the charge in the direction to progressively cool the same, providing temperature conditions of the charge such that any other volatile product escaping from the charge with the volatilized metal will be rendered incapable of oxidizing the volatile metal after escaping from the charge, and condensing the volatilized metal apart from the charge.

14. The method of smelting ores yielding a volatile metal which consists in heating a charge comprising carbon and proportioned to yield a fusible slag, conducting the volatilized reaction products through the charge, and maintaining a temperature of the charge such that any  $\text{CO}_2$  will be converted into  $\text{CO}$  before escaping from the charge.

15. The method of smelting ores yielding a volatile metal which consists in progressively feeding a charge into the smelting chamber, progressively supplying the charge with a layer of reducing material, heating a portion of the charge to smelting temperature, conducting the volatile products through the cooler portions of the charge and through the layer of reducing material, and condensing the metal apart from the charge.

16. The method of smelting zinc ores, which consists in electrically progressively heating, in the absence of extraneous air, a charge proportioned to yield a fusible slag, conducting the volatile reaction products through the charge and into contact with carbon heated to a reducing temperature, and condensing the zinc.

17. The method of smelting zinc ores, which consists in progressively heating, in the absence of extraneous air, a charge proportioned to yield a fusible slag, said charge comprising carbon, conducting the volatile reaction products through the charge and into contact with portions thereof heated to the temperature of maximum reductivity of carbon, and condensing the zinc apart from the charge.

In testimony whereof I affix my signature, in the presence of two witnesses.

WOOLSEY McA. JOHNSON.

Witnesses:

J. THOMSON,  
L. A. WATSON.

It is hereby certified that in Letters Patent No. 1,080,912, granted December 9, 1913, upon the application of Woolsey McA. Johnson, of Hartford, Connecticut, for an improvement in "Methods of Electrically Smelting Volatile Metals," an error appears in the printed specification requiring correction as follows: Page 5, line 97, for the word "as" read *gas*; and that the said Letters Patent should be read with this correction therein that the same may conform to the record of the case in the Patent Office.

Signed and sealed this 30th day of December, A. D., 1913.

[SEAL.]

J. T. NEWTON,

*Acting Commissioner of Patents.*